

# UNITED STATES PATENT OFFICE.

LEON DE WOLF WANTE, OF ST. NICOLAS-WAAS, BELGIUM.

DIVIDING, LANIFYING, AND BLEACHING BASS-FIBERS.

1,112,873.

Specification of Letters Patent.

Patented Oct. 6, 1914.

No Drawing.

Application filed September 7, 1912. Serial No. 719,142.

To all whom it may concern:

Be it known that I, LEON DE WOLF WANTE, a subject of the King of Belgium, and a resident of St. Nicolas-Waas, in Belgium, have invented certain new and useful Improvements in Dividing, Lanifying, and Bleaching Bass-Fibers, of which the following is a specification.

This invention relates to a novel process for dividing, lanifying and bleaching simultaneously bassfibers such as jute, hemp, flax, cocoa and other fibers that are obtained by steeping or retting. If the fiber is pure the division and lanification can be done easily with more or less concentrated alkali lye, but if the fiber is more or less lignified and therefore hard, caustic lye acts very slowly and sluggishly and the fiber turns brown. To overcome this deficiency it has been proposed to place the fiber after this treatment in the alkali bath into a bath of a hypochlorite of an alkali metal.

Now I have found that I can divide, lanify and bleach the bassfibers with a good result if the fiber is treated according to my invention, in a single bath composed of alkali lye and hypochlorite of sodium or potassium solution. I have obtained good results by composing my bath as follows: I mix one volume of caustic potash or caustic soda lye of 36° Bé. with one volume of hypochlorite of potassium or sodium solution of 20° Bé. It is unnecessary to heat this combination bath and it takes some- times only about 10 minutes to produce the desired effect, but of course the time used depends on the nature of the fiber. Sometimes the material has to be kept in the bath for 4 hours and even more. When the fiber has been treated long enough in the bath, it is pressed out and dried, or if found necessary, washed out first and then pressed and dried.

To give the fiber a greater softness and luster I can combine my process with a subsequent treatment in hot water to which is added for instance 1 per cent. of glycerin, soap, or soapoil, Turkey red oil or the like. The composition of the mixed bath may vary

according to the nature of the fiber to be treated for instance if the fiber to be treated is less lignified I can compose the bath of 3 parts by volume of caustic lye of 36° Bé. and of 7 parts by volume of hypochlorite of sodium or potassium of 12° Bé.

Having fully described my invention what I claim is—

1. The process of producing bleached and softened bassfibers, such as jute, hemp, flax, cocoa and the like fibers consisting in subjecting the steeped or retted fibers first to a bath composed of caustic alkali lye and a solution of an alkali metal salt of hypochlorous acid, and then softening the fibers.

2. The process of producing bleached and softened bassfibers, such as jute, hemp, flax, cocoa and the like fibers consisting in subjecting the steeped or retted fibers first to a bath composed of equal volumes of caustic alkali lye of 36° Bé. and of a solution of an alkali metal salt of hypochlorous acid of 20° Bé., and then softening the fibers.

3. The process of producing bleached and softened bassfibers, such as jute, hemp, flax, cocoa and the like fibers consisting in subjecting the steeped or retted fibers to a bath composed of caustic alkali lye and a solution of an alkali metal hypochlorite, pressing out or drying the fibers, and then subjecting them to a hot water bath containing a small percentage of a substance adapted to impart softness and luster.

4. The process of producing bleached and softened bassfibers, such as jute, hemp, flax, cocoa and the like fibers consisting in subjecting the steeped or retted fibers to a bath composed of caustic alkali lye and a solution of an alkali metal hypochlorite, pressing out or drying the fibers, and then subjecting them to a hot water bath containing about 1% of glycerin.

5. The process of producing bleached and softened bassfibers, such as jute, hemp, flax, cocoa and the like fibers consisting in subjecting the steeped or retted fibers to a bath composed of potash lye and a solution of an alkali metal hypochlorite, pressing out or

drying the fibers, and then subjecting them to a hot water bath containing about 1% of glycerin.

6. The process of producing bleached and softened bassfibers, such as jute, hemp, flax, cocoa and the like fibers consisting in subjecting the steeped or retted fibers to a bath composed of potash lye and a solution of hypochlorite of potassium, pressing out or

drying the fibers, and then subjecting them to a hot water bath containing about 1% of glycerin.

Signed at Cologne, Germany this 30th day of August 1912.

LEON DE WOLF WANTE.

Witnesses:

BERTHOLD FLEISCHER,  
LOUIS VANDORY.